

Feb. 11, 1941.

C. E. NELSON

2,231,023

METHOD OF TREATING MAGNESIUM

Filed Feb. 23, 1939

2 Sheets-Sheet 1



Fig. 1



Fig. 2

INVENTOR  
Charles E. Nelson

BY  
Griswold & Burdick  
ATTORNEYS

Feb. 11, 1941.

C. E. NELSON

2,231,023

METHOD OF TREATING MAGNESIUM

Filed Feb. 23, 1939

2 Sheets-Sheet 2



Fig. 3

INVENTOR  
Charles E. Nelson

BY  
Griswold & Burdick  
ATTORNEYS

## UNITED STATES PATENT OFFICE

2,231,023

## METHOD OF TREATING MAGNESIUM

Charles E. Nelson, Midland, Mich., assignor to The Dow Chemical Company, Midland, Mich., a corporation of Michigan

Application February 23, 1939, Serial No. 257,924

6 Claims. (CL 75—67)

This invention relates to the treatment of magnesium. It more particularly concerns a method of treating commercial magnesium whereby it is rendered highly pure or the magnesium in magnesium scrap, such as castings, alloys and the like, can be recovered in a highly pure state.

I have found that the presence of certain impurities in magnesium, even though these be present in very limited amounts, greatly accelerates the rate at which magnesium corrodes. For example, it is recognized that the presence of a small amount of iron in magnesium greatly accelerates the rate at which magnesium corrodes and may thus render it unsuitable for many commercial uses. The impurities nickel and copper affect the rate at which magnesium metal corrodes similarly.

To remove these impurities ordinarily present in the magnesium produced by present practices, it has heretofore been proposed to subject the magnesium to sublimation or distillation. However, I have observed that unless the metal being purified is subjected to repeated sublimation or distillation, as the case may be, the impurities are not generally removed to the extent that they no longer greatly accelerate the rate at which magnesium corrodes or otherwise adversely affect the properties of the metal. In some instances, even by repeated distillations or sublimations, the metal cannot be rendered satisfactorily pure.

It is, therefore, the principal object of the invention to provide a method of rendering magnesium so highly pure that the impurities no longer have substantially any adverse effect as regards the rate at which magnesium corrodes. Another object of the invention is to provide a method whereby magnesium can be rendered pure in a single operation. Other objects and advantages will be apparent as the description proceeds.

I have discovered that if the magnesium to be purified is caused to vaporize in the presence of a metal selected from the group of metals consisting of lead, tin, bismuth, calcium, silicon, and antimony, the impurities can be removed to the extent that the rate at which ordinary commercial magnesium corrodes is greatly reduced.

50 The invention then resides in the method hereinafter fully described and particularly pointed out in the claims, the accompanying drawing and following description setting forth in detail a mode of carrying out the invention, such mode illustrating, however, but one of various ways in

which the principle of the invention may be used.

In said drawing:

Fig. 1 is a sectional view in elevation of the apparatus.

Fig. 2 is a top plan view of said apparatus.

Fig. 3 is a view of the apparatus illustrated in Fig. 1 showing a slightly modified structure.

In the drawing an upright cylindrical iron retort 1 is shown closed at the bottom 17 and provided at the top end with a flange 2, to which is attached a gasket sealed head 3 by means of suitable bolts 4. Condenser 5, in the form of a section of iron pipe closed at its lower end is attached centrally to the interior side of head 15 10 and extends into the retort. Externally of the retort a cooling water inlet 6 and water outlet 7 communicate with the interior of the condenser 5. A mass of purified condensed magnesium 8 is shown clinging to the condenser 5. 20 A vacuum connection 9 communicates through head 3 with the interior of the retort and provides a means whereby the retort may be connected to a vacuum pump (not shown) and held under reduced pressure. A cooling coil 10 intimately attached to head 3 (as by welding) encircles the head directly above gasket 11 and serves to prevent the gasket from becoming overheated. Internally of the retort a removable iron charge container 12 partially filled with a 30 solid charge 13 consisting of a quantity of impure magnesium and a suitable metal added to effect the purification of the magnesium rests on the bottom of the retort. As a means of heating the retort, electrical leads 14 are connected to resistance wire 15 which encircles the lower portion of the retort. A suitable insulating material 16 surrounds the retort and serves to protect it from excessive heat loss due to radiation.

In the view illustrated in Fig. 3 the apparatus of Fig. 1 has been modified by suspending a shallow perforate metal basket 18 over charge container 12. The basket 18 is suspended from the charge container 12 by means of flange 19 which engages the top portion of charge container 12. 45 A perforate cover 20 is shown seated on top of the basket 18 and acts to confine the filter bed. Basket 18 serves as a container for a filtering material designated generally by numeral 21 in case such is used.

In carrying out the method of the invention, the iron container 12 is filled with a charge 13 consisting of impure magnesium and the added purifying metal and lowered into the retort through the open end. The retort is then closed 55

up by bolting flanged head 3 in place. Cooling water is then started through lines 6 and 7 and through coil 10 while vacuum is applied to exhaust the interior of the retort of gases through line 9. When the desired degree of vacuum is obtained, electric current is supplied to the resistance wire 15 through electrical leads 14 to heat the retort, care being taken in the meantime to maintain the vacuum. The impure magnesium as well as the added metal rapidly melts and, as magnesium vapor forms, it collects and condenses on the cold surface of condenser 5 where it adheres in the form of compact crystals. After such a time has elapsed as will indicate that substantially all of the magnesium has been distilled off, the current may be shut off, the vacuum broken, and the flange head detached from the retort. The magnesium crystals can then be stripped from the condenser. Additional impure magnesium may be immediately added to the charge container without removing the residue therefrom and the process of purifying metal continued.

As afore-mentioned, the metals suitable for use are the metals selected from the group of metals consisting of lead, tin, bismuth, calcium, silicon and antimony. If desired, mixtures of these metals may be suitably employed. For example, a particularly effective mixture consists of tin and lead. In general the amount of such metal to employ to effect the removal of undesirable impurities is from 10 to 50 per cent or more by weight, based upon the weight of the impure magnesium, and preferably between 25 to 35 per cent. It is unnecessary to remove the residue, consisting mainly of the added metal, from the charge container after every run, since in practice it has been found that as many as 20 or more charges of impure magnesium may be purified with but a single addition of the purifying metal.

It is usually desirable to operate under relatively high vacuum, as for example, less than 2 millimeters of mercury, and preferably below 0.2 of a millimeter, since under such highly reduced pressure the purified magnesium condenses out in the form of a dense compact mass rather than in the form of long needle-like crystals. Condensation in a dense compact form is desirable because relatively little surface area is exposed to oxidation when the metal is later rehandled for remelting or the like, in comparison with the area exposed when a needle-like crystal structure is produced. Operating at highly reduced pressure offers the additional advantage that the temperature required to effectively carry out the process is such that the apparatus may be constructed of readily available iron or steel without any danger of destruction due to the high temperature necessary if the purifying operation is carried out at higher pressure. If desired, a suitable inert gas may be introduced into the retort to prevent destructive attack by air or other gases upon the purified metal, although under the preferred vacuum conditions such procedure is unnecessary.

The temperature to be employed in the distillation or sublimation may, of course, be varied quite widely, as for example between about 500° to 800° C., depending however upon the degree of vacuum employed. At 0.05 millimeter pressure of mercury a temperature of 700° C. has been found highly satisfactory. It is preferable that the magnesium be caused to vaporize at

such a temperature that the added metal melts in the presence of the magnesium vapor.

The time required to purify a batch of metal also depends upon the amount of heat supplied to the metal as well as the pressure employed. In a retort such as illustrated, 16 inches in diameter, it is possible to distill off from three to four pounds of magnesium per hour by holding the temperature at about 700° C. and the pressure at 0.05 millimeter.

Although magnesium of a relatively high degree of purity and, therefore, highly resistant to corrosion can be produced in the manner above described I have made the further discovery that by using the present process in conjunction with a filtering operation, such as is disclosed in my co-pending applications Serial Nos. 257,923, filed February 23, 1939 and 257,871, filed February 23, 1939, magnesium of even a higher degree of purity can be obtained with a consistency that is not possible when employing either of the methods alone. In the above said co-pending applications there is disclosed and claimed methods of purifying magnesium either by causing the magnesium vapor to pass through a porous, granular, or fibrous filter bed of a refractory selected from the group of refractories consisting of the oxides and silicates located above manganese in the electromotive series of metals, or by causing the vapor to pass through a porous filter bed of a granular salt selected from the group of salts consisting of the halides of the alkali and alkaline earth metals. A purifying operation, wherein the magnesium vapor is passed through a filter bed of a refractory or a halide salt, as well as being vaporized in the presence of one of the metals, such as lead or the like, in the above described manner, is carried out by suspending the shallow perforate metal basket filled with a filtering medium over the charge container in such a manner that the magnesium vapor filters through the prepared bed. The depth of the filter bed so prepared is found to operate most effectively if it is between from 1/2 to 2 inches. The temperature and pressure conditions under which the combined processes may be operated satisfactorily are generally the same as for either process alone. In general, when employing a filter in combination with a metal, a smaller amount of the purifying metal gives satisfactory results. For example, when employing a metal alone, the preferred amount is from 25 to 35 per cent by weight. When employing the combined processes, from 15 to 25 per cent of the metal is generally preferable. A generally desirable combination to employ, because of the high degree of purity of the product obtained, is from 15 to 20 per cent by weight of lead in combination with a filter composed of rock wool.

Other modes of applying the principle of my invention may be employed instead of those explained, change being made as regards the method herein disclosed, provided the step or steps stated by any of the following claims or the equivalent of such stated step or steps be employed.

I therefore particularly point out and distinctly claim as my invention:

1. The method of producing substantially pure magnesium comprising bringing impure magnesium into direct contact with from 10 to 50 per cent by weight of a metal selected from the group of metals consisting of lead, tin, calcium, bismuth, antimony and silicon, applying heat so as

to cause the metals to alloy, and thereafter continuing the application of heat so as to cause the magnesium to vaporize from the so-alloyed mixture.

2. The method of producing substantially pure magnesium comprising bringing impure magnesium into direct contact with from 10 to 50 per cent by weight of a metal selected from the group of metals consisting of lead, tin, calcium, bismuth, 0 antimony and silicon, maintaining a vacuum on the metals while applying heat so as to cause the metals to alloy, and thereafter continuing the application of heat so as to cause the magnesium to vaporize from the so-alloyed mixture.

15 3. The method of producing substantially pure magnesium comprising bringing solid impure magnesium into direct contact with from 25 to 35 per cent by weight of a metal selected from the group of metals consisting of lead, tin, calcium, bismuth, 20 antimony and silicon, applying heat so as to cause the metals to alloy, continuing the application of heat so as to cause the magnesium to vaporize from the so-alloyed mixture while maintaining the metals under a pressure of less than 2 millimeters of mercury, and 25 thereafter condensing the magnesium vapor.

4. The method of producing substantially pure magnesium comprising introducing impure magnesium into direct contact with from 10 to 50 per cent by weight of a metal selected from the group 30 of metals consisting of lead, tin, calcium, bismuth, antimony and silicon, applying heat so as to cause the metals to alloy, continuing the ap-

plication of heat so as to cause the magnesium to vaporize, and thereafter passing the magnesium vapor through a filter bed of a solid granular salt selected from the group of salts consisting of the halides of the alkali and alkaline earth 5 metals.

5. The method of producing substantially pure magnesium comprising bringing impure magnesium into direct contact with from 25 to 35 per cent by weight of a metal selected from the group 10 of metals consisting of lead, tin, calcium, bismuth, antimony and silicon, applying heat so as to cause the metals to alloy, continuing the application of heat so as to cause the magnesium to vaporize while maintaining the metals under 15 highly reduced pressure, and thereafter passing the magnesium vapor through a filter bed of a solid salt selected from the group of salts consisting of the halides of the alkali and alkaline 20 earth metals.

6. The method of producing substantially pure magnesium comprising heating an alloy consisting of magnesium and from 10 to 50 per cent by weight of at least one of the metals selected from the group of metals consisting of lead, tin, calcium, bismuth, 25 antimony and silicon so as to cause the magnesium contained in the alloy to vaporize, passing the magnesium vapor through a filter bed of a solid granular salt selected from the group of salts consisting of the halides of the alkali and alkaline earth metals, and thereafter 30 condensing the magnesium vapor.

CHARLES E. NELSON.